

July 31, 1956

W. H. MOORE

2,756,476

PROCESS FOR IMPROVING THE PERMEABILITY-RAMMING  
CHARACTERISTICS OF FOUNDRY SAND

Filed Sept. 19, 1952

4 Sheets-Sheet 1

*Fig. 1*



*Fig. 2*



*Fig. 3*



INVENTOR.  
WILLIAM H. MOORE

BY Woodling and Krout  
attys

July 31, 1956

W. H. MOORE  
PROCESS FOR IMPROVING THE PERMEABILITY-RAMMING  
CHARACTERISTICS OF FOUNDRY SAND

2,756,476

Filed Sept. 19, 1952

4 Sheets-Sheet 2

*Fig. 4*



*Fig. 5*



July 31, 1956

W. H. MOORE

2,756,476

PROCESS FOR IMPROVING THE PERMEABILITY-RAMMING  
CHARACTERISTICS OF FOUNDRY SAND

Filed Sept. 19, 1952

4 Sheets-Sheet 3



WILLIAM H. MOORE  
BY Woodling and Kroft  
atlas

July 31, 1956

W. H. MOORE

2,756,476

PROCESS FOR IMPROVING THE PERMEABILITY-RAMMING  
CHARACTERISTICS OF FOUNDRY SAND

Filed Sept. 19, 1952

4 Sheets-Sheet 4

NATURAL BONDED SAND



Fig. 9



Fig. 10

INVENTOR.  
WILLIAM H. MOORE  
BY *Woodling and Kroet*  
*attys*

**1**

2,756,476

**PROCESS FOR IMPROVING THE PERMEABILITY-RAMMING CHARACTERISTICS OF FOUNDRY SAND**

William Henry Moore, Larchmont, N. Y., assignor to Meehanite Metal Corporation, a corporation of Tennessee

Application September 19, 1952, Serial No. 310,438

8 Claims. (Cl. 22—217)

This invention relates to foundry practice in general, and relates more particularly to control of molding sand characteristics for making sand castings.

This application is a continuation-in-part of application, Serial No. 173,853, filed July 14, 1950, for Foundry Sand Control, now abandoned.

An object of this invention is to provide a method of controlling the variations in a sand which are due to the varying properties resulting when a sand is rammed to varying degrees.

Another object of this invention is to provide a method of controlling the uniformity of a mold produced by ramming, and the subsequent uniformity of surface finish produced on a casting.

Still another object of this invention is to relate the degree of change of said permeability and degree of change of strength to a theoretical ideal, and to one another.

Other objects and a fuller understanding of the invention may be had by referring to the following description and claims, taken in conjunction with the accompanying drawings, in which:

Figure 1 is a curve plotted from one given sand by testing the permeability over a variation in ramming;

Figure 2 is a diagrammatic representation of the reason why one given sand will pack more than another under ramming;

Figure 3 is a curve of several sands, plotted as in Figure 1, but each sand having different beginning and ending permeabilities at various levels;

Figure 4 is a graph of one sand plotting green compression strength variations in relationship to number of rams in a laboratory test sample;

Figure 5 is a graph of several sands plotted on the same coordinates as Figure 4, but each sand having different beginning and ending strengths, and each at a different level;

Figure 6 is a test mold, and the pattern for producing the mold;

Figure 7 is a graph plotting percentage of variation in mold hardness to percentage of ramability to illustrate the decrease in mold hardness variance with increase in ramability percentage;

Figure 8 is a graph showing vertical columns to illustrate the percentage of castings scrapped due to a defect, as compared to the percentage of ventability, with a dotted angular line illustrating the trend of decrease with increase of ventability percentage;

Figure 9 is a graph plotting percentage, ventability and bondability against moisture content in order to illus-

**2**

trate how these properties may be changed by varying the moisture content; and

Figure 10 is a graph showing the variation in mold hardness obtained in a test mold with different degrees of ramming and varying the values in ventability and bondability.

The preparation of a mold for casting metal has long been subject to many variables, particularly those variables due to uneven ramming or packing of the sand around the pattern. Thus in ramming by hand, for example, certain areas of the mold will always be rammed harder than other areas, and the resultant mold will not be uniform in its behavior towards the molten metal that is subsequently introduced into it. Where the ramming is soft, mold surface will be weak and porous, and the appearance of the casting at this point will be rough and uneven. When the ramming is hard the casting may contain defects due to the inability of the metal to lie quietly on a hard surface of high density.

20 The introduction of mechanical methods of ramming molds has done little to improve this situation, as the uniformity of ram is very largely dependent on the design of the mold cavity and the molding sand is unable to pack firmly in narrow pockets and the like. In the past, with a 25 skillful hand ram it was possible to carefully pack the sand in these narrow pockets and thereby present a mold of fairly uniform properties. However, this peening operation requires more than average skill on the part of the operator and is time-consuming, so it has little place 30 in the modern methods of manufacture.

This problem of obtaining a uniform mold surface by the ramming of sand has been given considerable attention in the past, but with little success. One such means has been to use a hardness tester on the molds in order 35 to investigate the relative hardness at any particular spot in the mold. If this hardness was adjudged to be too low, then the ramming was increased. However, an increase in ramming increases the hardness at the spot under discussion and also increases the hardness at other portions 40 of the mold. This method therefore does not improve the uniformity of hardness over the mold surface. The hardness can be raised and lowered by alteration in the degree of ramming, but the different hardness values in different areas of the mold cannot be substantially 45 avoided by this means.

In order to make a commercially salable casting free from blemishes and defects, a mold surface must have two very definite properties at a suitable level. It must 50 have strength and rigidity to resist the fluid pressure of the molten metal, and it must have permeability to dissipate steam and other gases. Too low a strength will lead to collapse of the mold surface and too high a strength may cause contraction strains and even cracks 55 in the casting. Too high a permeability will give a rough, uneven surface to the casting, and too low a permeability will lead to blows, scabs and many other common casting defects.

It has been generally recognized that the permeability 60 and the strength of a mold sand will vary according to the degree to which the sand is rammed, and according to the type and amount of bonding agent, as well as the amount of actual temper moisture present. Thus, as we ram harder we will increase the strength and decrease the permeability. It had not heretofore been

realized, however, that the amount of change in these properties with ramming is capable of measurement and control in such a manner that a uniformly hard mold may be produced regardless of the degree and method of ramming employed.

The problem is to provide a mold of uniform permeability and of uniform strength across the whole surface. If this condition is present, it follows that a casting of uniform character can be produced. After considering this problem from many different standpoints, it was realized that if a sand were of such a nature that it did not change in permeability, or in strength, as it was rammed from a relatively soft degree of ram to a relatively hard degree of ram, it would automatically give a uniform mold irrespective of the method or degree of ramming.

Laboratory measurements of permeability and of strength involve the preparation of a standard sample 2 inches in diameter and 2 inches high. This sample is rammed three times by dropping a weight of 14 pounds through a height of 2 inches on the sand. This is a standard ram, and it has long been realized that this standard degree of ramming used in the laboratory is not fully representative of the average degree of ramming used in a foundry. Each method of ramming in the foundry is either lesser or greater than the standard ram, depending on whether the ramming is a hand operation, a jolt operation, a jolt-squeeze operation, or a slinger operation.

As the result of a long experience in the different methods of ramming and in the art of producing foundry molds and cores, I have been able to establish a ramming range in the laboratory manner which will adequately represent the degree of ramming obtained with normal methods of ramming used in production. Thus, if I ram a sand in the laboratory at one ram or one drop of the weight as a minimum, and 10 rams or 10 drops of the weight as a maximum, I will have conditions representing and including the softest and the hardest rams usually found in practice.

I do not wish to limit myself strictly to this range of ramming. I have chosen this range of ramming as being representative of the average range found in practice, but the method of testing which I will describe hereafter can just as easily be applied to a degree of ramming considerably wider than this 1-10 ram range. Thus, I could select a range of 1-2 rams or 1-100 rams in order to include some unusual method of ramming in practice. I could also change the 14-pound weight used to any other value and I could prepare the samples by different methods of ramming. The standard method of sample preparation has been chosen as a basis of measurement merely because of convenience. In the same way, the range of 1 to 10 rams on the standard rammer has been chosen merely because it is reasonably representative and includes most normal degrees of ramming or hardness found in practice.

My testing method involves relating the degree of variance of permeability and of strength with variance in ramming to an ideal condition. An ideal condition or an ideal sand is one which does not change in permeability, or in strength over the complete range of ramming chosen for testing purposes.

Reference to Figure 1 shows a graph which records the tests conducted on a molding sand. The lowering of permeability with increase in ramming can readily be observed. On the same graph the broken lines represent theoretically ideal sands which retain their properties at the same level throughout the ramming range. These ideal sands are shown at different levels of property values to emphasize that the only requisite of an ideal sand is no change in properties with ramming. It matters little whether these properties are at a high level or at a low level insofar as designating them as ideal sands. Ideal simply means that there would be no change in permeability regardless of the number of rams,

One particular ideal sand may not be a suitable sand for a given mold, although it could be. If the ideal level falls at a strength that is too high or too low, or at a permeability level which is too high or too low, or both, then a good casting will not result, regardless of the fact that the sand is an ideal sand and does not change its characteristics with additional ramming.

It should be emphasized that progressive ram tests are by no means new and have been conducted by many sand technicians in an effort to differentiate between the behavior of various sands. However, the tests are always at an arbitrary standard, not related to actual foundry practice. Further, and by far the greatest failure, these tests stand alone as academic facts, unrelated in any way to actual foundry practice. It is a well-known fact, until the time of this invention, that laboratory test data on sand are of little practical value, and that usually the foundry foreman will alter his sand by some hunch or guess, often based upon reasoning amounting almost to superstition.

This invention is based upon the fact illustrated graphically in Figure 2, together with the selection and alteration of a foundry sand having a combination of permeability and strength factors related to one selected ideal sand, and to one another.

Figure 3 illustrates two facts which were heretofore apparent, but which were never used in a process of selecting and blending a satisfactory mold sand, as this invention now teaches. Figure 3 is a chart showing several curves resulting from plotting permeability changes with respect to the number of rams in a standard controlled laboratory test. In each case the permeability of the sand decreases with increasing ramming. This fact is expected, and is explainable by the Figure 2. Bonding material and moisture are further factors affecting permeability, but in any event a given sand will produce a test curve, or any sand may be compounded and altered to produce a variety of curves.

From Figure 3, the fact is apparent that not any degree of permeability can be obtained from one sand. Some sands, however, give a much wider span of values, resulting in a graph more like Figure 1.

To be certain that the reason is understood for former failure of laboratory sand testing as a guide, let it be assumed that the foundry technician knows that a sand having a permeability of 130 (arbitrary scale) is satisfactory for his job. This knowledge that a permeability is satisfactory is an empirical knowledge. At the present time, there is no certain way to predetermine by scientific means just what permeability is required for any given casting problem.

The technician then conducts a laboratory sand test consisting of three rams by a 14-pound weight on a standard size sample. Assume that the sand which was tested to produce the graph of Figure 1 was the one selected. The test would show this sand to be acceptable. At three rams, graph Figure 1 shows substantially a permeability of 130.

But in the foundry this sand would produce many bad castings. The ramming in the foundry is never uniform, regardless of the type or quality of ramming machine available. Therefore, the mold maker may have ample time available at one time of the day, and he will then give each mold a full measure of ramming. In that event the actual mold permeability of the sand of Figure 1 will be considerably less than 130, maybe as low as 60, thereby producing a dense mold. The same operator, at another time, may be in a hurry and ram only enough to form the surface. This quick ram may then be only equivalent to a laboratory sample of one or two rams. Figure 1 sand then would have a permeability of 160 or 180 or more. Obviously, then, a standard ram test, standing alone, will reveal nothing of usefulness. An ideal sand having a permeability of 130

would solve the permeability problem, if such a sand were available.

The first discovery of this invention, therefore, is the reason why standard permeability tests, standing alone, are of little or no value.

After this first discovery, one may conclude that the logical solution to the production of a desired permeability would be to control the ramming. But that solution is not satisfactory, especially in view of the human element involved. Adjustment of the average sand grain size and type, bonding material, and temper moisture, by additions to a sand, or the compounding of a new sand mix, for producing a sand more nearly like an ideal sand, is the better solution of the problem of permeability. But the more nearly a sand mix approaches an ideal condition, the less range of permeability it includes; therefore, the less universal in application it becomes. Accordingly, there is both a theoretical and practical limit in the approach toward an ideal sand.

Figure 4 is a study similar to Figure 1, taking into consideration the green compression strength of a sand with respect to the number of rams. Here the strength increases with increase in ramming. It is almost impossible to designate an ideal strength value, because of the many factors involved, but an ideal sand with respect to strength would be a sand which did not change in strength over a wide range of ramming, as shown by the straight broken lines of Figure 4. The Figure 5 shows a group of sands which have strength curves more nearly approaching ideal than the sand of Figure 1.

As explained above, an ideal sand which does not vary in properties as it is rammed progressively harder will give a mold of uniform properties in practice regardless of the degree of ramming used in practice. Such a sand would be 100 per cent with respect to freedom from permeability variance and with respect to freedom from strength variance.

For the sake of identification and ease of expression, the degree of variation in permeability with variation in ramming is called the "ventability," and the degree of variation in strength with variation in ramming is called the "bondability." On this method of nomenclature an ideal sand would have 100 per cent ventability and 100 per cent bondability. The terms ventability and bondability may be used by others, and if so are not to be given any general meaning in this field. Rather, these terms are intended to be limited strictly to the definitions just given.

From the foregoing discussion, it is apparent that the discoveries of sand behavior disclosed would be useful in reducing casting defects, if no further use were made of this information. However, if properly understood and applied, this information can be further utilized to perfect sand practice at the foundry level.

The foregoing discussion has disclosed the possible variations in sand behavior, and explained what an ideal sand would be. The actual sands produce a graph differing from the ideal sand. This difference can be related to the ideal, and a percentage value of the variation of permeability curves from the ideal of 100 per cent may be obtained.

By the same token, the percentage value of the variation of the strength curves from the ideal of 100 per cent may be obtained.

The mechanics, or mathematics, of relating actual sands to ideal standards is explained hereafter. But it is the fact of relating that is believed to constitute the basic invention, not the specific mathematical method given. However, this specific method is new, inasmuch as it is part and parcel of the new basic discovery of said behavior, and its relationship to an idea.

We can now proceed to actually express and measure the ventability and the bondability of any molding or core sand simply by reference to an ideal sand. Consider, for example, the test given in Figure 1. At the

first ram the sand has a permeability of 210. If it had 100 per cent ventability, it would show this same value of 210 over the complete ramming range. If now we set this ideal condition down in tabular form and divide each permeability value by the succeeding one we will have the following:

### PERMEABILITY

|    | No. of Rams | Permeability | Sub-Total                                       |
|----|-------------|--------------|-------------------------------------------------|
| 15 | 1.....      | 210          | $P \text{ at } R_1 = \frac{210}{210} = 1.00$    |
|    | 2.....      | 210          | $P \text{ at } R_2 = \frac{210}{210} = 1.00$    |
|    | 3.....      | 210          | $P \text{ at } R_3 = \frac{210}{210} = 1.00$    |
| 20 | 4.....      | 210          | $P \text{ at } R_4 = \frac{210}{210} = 1.00$    |
|    | 5.....      | 210          | $P \text{ at } R_5 = \frac{210}{210} = 1.00$    |
|    | 6.....      | 210          | $P \text{ at } R_6 = \frac{210}{210} = 1.00$    |
| 25 | 7.....      | 210          | $P \text{ at } R_7 = \frac{210}{210} = 1.00$    |
|    | 8.....      | 210          | $P \text{ at } R_8 = \frac{210}{210} = 1.00$    |
| 30 | 9.....      | 210          | $P \text{ at } R_9 = \frac{210}{210} = 1.00$    |
|    |             |              | $P \text{ at } R_{10} = \frac{210}{210} = 1.00$ |
|    |             |              | Total..... 9.00                                 |

Where: P=permeability; R=ram number.

The same procedure may then be applied to the data in Figure 4. At the first ram a strength of 2.5 is shown. If this sand had 100 per cent bondability, it would show this same strength value at all rams over the test range.

40 The tabular relationship is as follows:

### STRENGTH

|    | No. of Rams | Strength | Sub-Total                                       |
|----|-------------|----------|-------------------------------------------------|
| 45 | 1.....      | 2.5      | $S \text{ at } R_2 = \frac{2.5}{2.5} = 1.00$    |
|    | 2.....      | 2.5      | $S \text{ at } R_1 = \frac{2.5}{2.5} = 1.00$    |
| 50 | 3.....      | 2.5      | $S \text{ at } R_3 = \frac{2.5}{2.5} = 1.00$    |
|    | 4.....      | 2.5      | $S \text{ at } R_4 = \frac{2.5}{2.5} = 1.00$    |
| 55 | 5.....      | 2.5      | $S \text{ at } R_5 = \frac{2.5}{2.5} = 1.00$    |
|    | 6.....      | 2.5      | $S \text{ at } R_6 = \frac{2.5}{2.5} = 1.00$    |
| 60 | 7.....      | 2.5      | $S \text{ at } R_7 = \frac{2.5}{2.5} = 1.00$    |
|    | 8.....      | 2.5      | $S \text{ at } R_8 = \frac{2.5}{2.5} = 1.00$    |
|    | 9.....      | 2.5      | $S \text{ at } R_9 = \frac{2.5}{2.5} = 1.00$    |
| 65 | 10.....     | 2.5      | $S \text{ at } R_{10} = \frac{2.5}{2.5} = 1.00$ |
|    |             |          | Total..... 9.00                                 |

Where: S=strength; R=ram number.

70 In these ideal cases the total of the quotients equals 9.00 which would be equivalent to 100 percent ventability and 100 per cent bondability. It must be remembered that there is no significance in the value of 9.00 apart from the illustration given.

If now we set down in tabular form the actual results

obtained with the sand depicted in Figure 1 and Figure 4, we have the following:

## PERMEABILITY

| No. of Rams | Permeability                                       | Sub-Total |
|-------------|----------------------------------------------------|-----------|
| 1.          | 210<br>$P \text{ at } R1 = \frac{210}{160} = 1.31$ |           |
| 2.          | 160<br>$P \text{ at } R2 = \frac{160}{130} = 1.23$ |           |
| 3.          | 130<br>$P \text{ at } R3 = \frac{130}{106} = 1.22$ |           |
| 4.          | 106<br>$P \text{ at } R4 = \frac{106}{90} = 1.18$  | 15        |
| 5.          | 90<br>$P \text{ at } R5 = \frac{90}{78} = 1.16$    |           |
| 6.          | 78<br>$P \text{ at } R6 = \frac{78}{70} = 1.11$    |           |
| 7.          | 70<br>$P \text{ at } R7 = \frac{70}{62} = 1.13$    | 20        |
| 8.          | 62<br>$P \text{ at } R8 = \frac{62}{60} = 1.03$    |           |
| 9.          | 60<br>$P \text{ at } R9 = \frac{60}{58} = 1.04$    | 25        |
| 10.         | 58<br>Total.....                                   | 10.41     |

Where: P=permeability; R=ram number.

## STRENGTH

| No. of Rams | Strength                                               | Sub-Total |
|-------------|--------------------------------------------------------|-----------|
| 1.          | 2.5<br>$S \text{ at } R2 = \frac{3.9}{2.5} = 1.56$     |           |
| 2.          | 3.9<br>$S \text{ at } R3 = \frac{5.0}{3.9} = 1.28$     |           |
| 3.          | 5.0<br>$S \text{ at } R4 = \frac{6.2}{5.0} = 1.24$     | 40        |
| 4.          | 6.2<br>$S \text{ at } R5 = \frac{7.2}{6.2} = 1.16$     |           |
| 5.          | 7.2<br>$S \text{ at } R6 = \frac{8.1}{7.2} = 1.12$     |           |
| 6.          | 8.1<br>$S \text{ at } R7 = \frac{8.8}{8.1} = 1.09$     |           |
| 7.          | 8.8<br>$S \text{ at } R8 = \frac{9.6}{8.8} = 1.09$     |           |
| 8.          | 9.6<br>$S \text{ at } R9 = \frac{10.2}{9.6} = 1.06$    | 50        |
| 9.          | 10.2<br>$S \text{ at } R10 = \frac{10.6}{10.2} = 1.04$ |           |
| 10.         | 10.6<br>Total.....                                     | 10.64     |

Where: S=strength; R=ram number.

If we now substitute these totals in the following formula:

Percent ventability or bondability=

$$\frac{9.0 - (\text{total} - 9.0)}{9.0} \times 100$$

or

$$\text{percent ventability or bondability} = (18.0 - \text{total}) \times 11.11$$

Then in the case of the theoretically ideal sand we will have:

$$\text{percent ventability or bondability} = (18.0 - 9.0) \times 11.11 = 100\%$$

Or, in the case of the sand shown in Figure 1 we will have:

$$\text{percent ventability} = (18.0 - 10.41) \times 11.11 = 84.24\%$$

And the sand shown in Figure 4 will have:

$$\begin{aligned} \text{percent bondability} &= (18.0 - 10.64) \times 11.11 \\ &= 81.70\% \end{aligned}$$

It has now been demonstrated how the change in properties with change in ramming of a sand may readily be related to a theoretically ideal condition. The mathematics of this method are not of importance, for on certain sands it will be found that the changes in properties with ramming are an exact logarithmic function and the same relationship to the ideal condition may be expressed by the use of logarithms. Also, as previously explained, the ramming range may be changed to suit any condition. If the two properties of permeability and strength are now considered together, we may say that where neither the permeability nor the strength changes with ramming change, we have a sand with a rammability of 100 percent. Again this term is chosen merely for convenience of expression and we say then that:

$$\text{percent rammability} = \text{percent ventability} + \text{percent bondability} = 2$$

Or this may be expressed in a single formula thus:

$$\begin{aligned} \text{percent rammability} &= 36 - (\text{total perm.} \\ &+ \text{total strength}) \times 5.556 \end{aligned}$$

The explanation of this method of evaluation has been dealt with in considerable detail not to illustrate the mathematics of relating sand properties to an ideal condition, but merely to illustrate that the sand properties may quite easily be related to our ideal condition. If now we again consider the original inventive thought, that an ideal sand, from a property change standpoint, must give a mold of uniform properties, irrespective of the degree and method of ramming, we can readily appreciate the basis of this invention. The same inventive thought can be applied quite readily to any other property of a molding sand which might vary with degree or intensity of ram. The properties of permeability and strength were chosen merely because they have a relatively great influence on the final casting produced from any mold.

Having thus shown how the "rammability" of a sand may be accurately evaluated, I am in a better position to demonstrate that these functions which I have called for convenience ventability, bondability and rammability, have a tremendous influence on the quality of castings produced in sand molds, and that by controlling these functions to definite limits I am able to overcome many of the problems which have long been a source of difficulty and expense to the foundry industry.

Practical use of this method of evaluation and control of these properties described as "ramming properties" over a period of time has quite conclusively demonstrated their far-reaching effects on casting quality and has aided very materially in the control of molding sands. Proper use of the teaching given herein will result in freedom from casting defects heretofore unknown. Defects due to defective molds has long been the foundryman's biggest problem. Therefore, this invention provides the solution to one of the most baffling problems. Actual experience in using the principles of this invention over considerable time of experimentation and study has proven the principles given to be sound, and of inestimable value.

The scope of this method of sand control may readily be appreciated from the following examples:

## Uniformity of molds

The effect of rammability on mold uniformity may be seen clearly in Figures 6 and 7. Figure 7 is a plotted curve of a sand showing the relationship of variation of hardness of various sands rammed in the mold of Figure 6 with respect to percent of rammability. A test mold is depicted in Figure 6 which was rammed under standard

conditions with the pattern having the dimensions shown. Hardness measurements were made on the face of the mold at points A, B, C and D. These measurements were averaged to give an average mold hardness for the complete mold, and the difference was taken between the highest reading and the lowest reading. The percentage variation of mold hardness was taken as the difference between the highest reading and the lowest reading divided by the average reading times 100.

A mold was rammed from different sands having different values of rammability.

The graph shows definitely that as the rammability approaches the ideal condition of 100 percent rammability, the variation in mold hardness is materially reduced. Thus we can readily control mold hardness variation by controlling the rammability of the sand used for making the mold.

The uniformity of surface finish on the castings improved directly with the improvement in rammability.

#### *Decrease in casting defects*

The ram properties can be used in reducing and elimination of defects due to sand. This is illustrated quite clearly in Figure 8, which shows the relationship between ventability and percent of castings scrapped due to scab defects. This graph was plotted from results over several months of operation in a foundry making a particular casting under controlled conditions, but where the ram properties were not under control. Subsequent control of the ventability to desirable limits eliminated these costly scab defects.

#### *Improvement in casting surface finish*

The ram properties can be used in the improvement of casting surface finish. It follows that if the molds can be made uniform by means of these properties, a uniform surface finish will result on all areas of a casting. By selecting a sand having sufficient smoothness to give a good surface and then making this sand having high ventability and bondability, it is possible to reproduce this smooth surface in the casting under a wide range of ramming conditions.

#### *Ramming of molds*

It has been shown that increasing uniformity of mold properties may be obtained by having the sand at a suitably high ventability and bondability value. It follows, therefore, that for any fixed method of ramming, the mold properties may be varied by changing the ventability and bondability. By the same token, the same uniformity of mold properties may be obtained in two cases in the following manner:

In case 1, the sand has a low ventability and bondability and the ramming is made excessively hard in order to overcome the natural reluctance of the sand to conform to the ideal condition.

In case 2, the ventability and bondability are high and a lesser degree of ramming is necessary to make this sand conform to the ideal condition. By increasing ventability and bondability, therefore, a mold of uniform properties may be obtained with a lower degree of ramming. We have, therefore, an excellent means of decreasing the power, energy and time necessary to make a mold of given uniformity. This, of course, leads to increased production and decreased molding costs. This concept is illustrated in Figure 10 showing the variation in hardness values obtained with a test casting.

Reference to Figure 10 shows that for the same percentage of variation in mold hardness, for example 30, the ramming degree used is less in the case of the sand having the highest ram properties. This means that by increasing the rammability of the sand mix used, it is possible to maintain an acceptable mold uniformity using a lesser ramming force. By doing this, great economies

in molding time and increase in production may be obtained.

It has been established by the disclosure given that every sand exhibits a degree of permeability change and a degree of strength change with variation in degree of ramming. These degrees of change are measurable and have been called the ventability and the bondability respectively. The combination of both the permeability change and the strength change has been called the rammability.

It has also been shown that these properties designated ventability, bondability and rammability may be used to increase mold uniformity and decrease casting defects. Anyone skilled in the foundry art knows that certain permeability values and certain strength values in their sand normally give them suitable castings. This knowledge is purely empirical and is based on years of bitter experience usually by trial and error. The reason that it is so difficult to establish a definite value of strength or permeability that will give an acceptable casting is because the strength and permeability that we actually obtain in a mold is not necessarily the same as that which we obtain in a laboratory test.

My invention enables us for the first time to translate laboratory test values of permeability and strength directly to the mold. This is done because under my invention we compound a sand mixture which does not vary in properties as the degree of ramming is varied. Consequently, we are able to eliminate the degree of ramming variable. This has never been done before.

In this particular invention, we are interested in providing a sand that will give us a uniform permeability and uniform strength in any mold that is made from the sand, irrespective of the method used in making the mold. We must assume that anyone skilled in the art will select a sand that will give a good level of properties in the mold calculated to give a good casting.

It now remains to be shown by specific example that the properties of ventability, bondability and rammability are capable of finite control. They may be varied by anyone skilled in the art to give the desired values necessary for the production of any particular casting or mold.

It was illustrated in Figure 8 that a lower defective loss due to scabs resulted when the ventability was higher. If in this case the economically accepted defective loss on these castings was 2%, it is obvious that a ventability above 86% is necessary in the manufacture of these castings.

The inclusion of ventability in the castings discussed in Figure 8 was necessary because conventional sand properties such as permeability and strength failed to show any means of reducing the high defective loss. This is because the test values of permeability and strength obtained in the sand used was not translated to the mold. In other words, no provision was made for the variation in properties of the sand as the degree of ramming varied. By allowing for this variation in properties with degree of ramming in the form of a ventability measurement, it was found that the actual molds could be made to give serviceable castings.

If now, the sand in this particular case is found to have a ventability of 82% with consequent higher than allowable defective loss, the problem is to increase the ventability of the sand to the acceptable 86% figure. This sand could be corrected in a series of steps, thus:

#### STEP 1

Examine the grain distribution of the sand by conducting a sieve analysis. If the grain is spread over a large number of sieves, it will give a low ventability. If it is confined with the greatest percentage on a relatively few adjacent sieves, it will give a higher ventability. By deliberately changing the distribution, therefore, the ventability may be altered as desired. By way of ex-

ample, a sand mixture having the following grain analysis gave ventability of 82.5%.

|               | Percent |
|---------------|---------|
| 20 mesh       | 0.2     |
| 30 mesh       | 0       |
| 40 mesh       | 0.2     |
| 50 mesh       | 21.8    |
| 70 mesh       | 36.0    |
| 100 mesh      | 18.6    |
| 140 mesh      | 10.6    |
| 200 mesh      | 0.6     |
| Pan           | 2.2     |
| Clay and silt | 7.2     |
| Ventability   | 82.6    |

It should be noted that 87.0% of the grains are on four adjacent screens. By changing the distribution to give approximately the same percentage of grains on three adjacent screens a ventability of 84.6% resulted, thus:

|               | Per cent |
|---------------|----------|
| 20 mesh       | 0.2      |
| 30 mesh       | 0.1      |
| 40 mesh       | 0.5      |
| 50 mesh       | 25.9     |
| 70 mesh       | 38.3     |
| 100 mesh      | 22.2     |
| 140 mesh      | 3.0      |
| 200 mesh      | 0.4      |
| Pan           | 2.1      |
| Clay and silt | 7.3      |
| Ventability   | 84.6     |

In the specific example quoted the change in grain distribution would not be sufficient to give the desired ventability. In such a case we would proceed with Step 2.

#### STEP 2

Examine the clay content of the sand mixture and reduce this for increased ventability.

By way of example, the ventability of sand mix was found to be 84.3%. This mix was as follows:

|           | Pounds |
|-----------|--------|
| Heap sand | 800    |
| New sand  | 160    |
| Sea coal  | 10     |
| Fireclay  | 30     |

The measured clay content was 5.3% by the hydrometer method. The mix was changed to:

|           | Pounds |
|-----------|--------|
| Heap sand | 800    |
| New sand  | 180    |
| Sea coal  | 10     |
| Fireclay  | 10     |

The measured clay content of the new mix was 4.2% and the ventability was 86.3%.

If Step 2 did still not result in the desired change we would proceed with Step 3.

#### STEP 3

Examine the moisture content of the sand and reduce this for increased ventability. This method of control has been described in the companion application bearing the Serial No. U. S. 173,852 and entitled "Optimum Temper Moisture Determination in Foundry Sand." In Figure 9 the variation in both ventability and bondability with moisture content on a typical sand mix is illustrated. By determining this data for the sand mix under consideration, it becomes possible to select the moisture value that will give the ventability, bondability or ram-ability desired.

In addition to the three steps outlined, there are other means of changing the ventability, bondability or ram-ability to any desired value. These means are tabulated as a general directive below and anyone skilled in the art

will automatically select the best course of procedure to follow rather than going through specific steps as outlined.

To raise ventability:

- Use a finer grain as long as the resultant permeability will fall within the desired limits.
- Use a round type of grain rather than the sub-angular type.

c. Decrease the bondability. If this results in too low a strength for normal operation, obtain fuller development of available bondability by the use of a small amount of Bentonite and by increased mulling.

d. Decrease the plasticity of the bond.

To raise bondability:

- Use a lightly coarser grain.
- Use a more rounded grain.
- Decrease the amount of bond or decrease the plasticity of the bond.

The opposite conditions will give the reverse of the effect anticipated and serve as directives for lowering the ventability and the bondability.

Although the invention has been described in its preferred form with a certain degree of particularity, it is understood that the present disclosure of the preferred form has been made only by way of example and that numerous changes in the details of construction and the combination and arrangement of parts may be resorted to without departing from the spirit and the scope of the invention as hereinafter claimed.

What is claimed is:

1. A process for improving the permeability-ramming characteristics of a foundry sand to obtain a predetermined permeability-change factor, said process comprising the steps of, providing a supply of foundry sand, test ramming and measuring the permeability-change between a first and second degree of ramming hardness of an initial sample-portion of said sand, physically altering the permeability-ramming characteristics of said sand until a subsequent sample-portion of altered sand shows substantially said predetermined permeability-change factor between said same first and second degrees of ramming hardness.

2. A process for improving the permeability-ramming characteristics of a foundry sand to obtain a predetermined permeability-change factor, said process comprising the steps of, providing a supply of foundry sand, test ramming and measuring the permeability-change between a first and second degree of ramming hardness of an initial sample-portion of said sand, physically altering the permeability-ramming characteristics of said sand by changing the grain size distribution of said sand until a subsequent sample-portion of altered sand shows substantially said predetermined permeability-change factor between said same first and second degrees of ramming hardness.

3. A process for improving the permeability-ramming characteristics of a foundry sand to obtain a predetermined permeability-change factor, said process comprising the steps of, providing a supply of foundry sand, test ramming and measuring the permeability-change between a first and second degree of ramming hardness of an initial sample-portion of said sand, physically altering the permeability-ramming characteristics of said sand by changing the bond-content of said sand until a subsequent sample-portion of altered sand shows substantially said predetermined permeability-change factor between said same first and second degrees of ramming hardness.

4. A process for improving the permeability-ramming characteristics of a foundry sand to obtain a predetermined permeability-change factor, said process comprising the steps of, providing a supply of foundry sand, test ramming and measuring the permeability-change between a first and second degree of ramming hardness of an initial sample-portion of said sand, physically altering the permeability-ramming characteristics of said sand by changing the moisture content of said sand until a subse-

## 13

quent sample-portion of altered sand shows substantially said predetermined permeability-change factor between said same first and second degrees of ramming hardness.

5. A process for improving the strength-ramming characteristics of a foundry sand to obtain a predetermined strength-change factor said process comprising the steps of, providing a supply of foundry sand, test ramming and measuring the strength-change between a first and second degree of ramming hardness of an initial sample-portion of said sand, physically altering the strength-ramming 10 characteristics of said sand until a subsequent sample-portion of altered sand shows substantially said predetermined strength-change factor between said same first and second degrees of ramming hardness.

6. A process for improving the strength-ramming characteristics of a foundry sand to obtain a predetermined strength-change factor said process comprising the steps of, providing a supply of foundry sand, test ramming and measuring the strength-change between a first and second degree of ramming hardness of an initial sample-portion 15 of said sand, physically altering the strength-ramming characteristics of said sand by changing the grain size distribution of said sand until a subsequent sample-portion of altered sand shows substantially said predetermined strength-change factor between said same first and 20 second degrees of ramming hardness.

7. A process for improving the strength-ramming char-

## 14

acteristics of a foundry sand to obtain a predetermined strength-change factor said process comprising the steps of, providing a supply of foundry sand, test ramming and measuring the strength-change between a first and second degree of ramming hardness of an initial sample-portion of said sand, physically altering the strength-ramming characteristics of said sand by changing the bond content of said sand until a subsequent sample-portion of altered sand shows substantially said predetermined strength-change factor between said same first and second degrees of ramming hardness.

8. A process for improving the strength-ramming characteristics of a foundry sand to obtain a predetermined strength-change factor, said process comprising the steps of, providing a supply of foundry sand, test ramming and measuring the strength-change between a first and second degree of ramming hardness of an initial sample-portion of said sand, physically altering the strength-ramming characteristics of said sand by changing the moisture content of said sand until a subsequent sample-portion of altered sand shows substantially said predetermined strength-change factor between said same first and second degrees of ramming hardness.

## References Cited in the file of this patent

Diertert: "Foundry Core Practice," second edition, pages 424-429, published 1950.